# EUROPEAN PATENT SPECIFICATION

(11) **EP 3 380 638 B1**
(45) Date of publication and mention of the grant of the patent: **11.03.2020**
(21) Application number: 16816320.2
(22) Date of filing: 23.11.2016
(51) Int. Cl.: C22B 47/00

(54) **METHOD AND APPARATUS FOR PREHEATING AND SMELTING MANGANESE ORE SINTER**
VERFAHREN UND VORRICHTUNG ZUM VORWÄRMEN UND SCHMELZEN VON MANGANERZSINTER
PROCÉDÉ ET APPAREIL DE PRÉCHAUFFAGE ET DE FUSION DE MINERAI DE MANGANÈSE FRITTÉ

(30) Priority: 24.11.2015 FI 20155868
(43) Date of publication of application: 03.10.2018
(73) Proprietor: Outotec (Finland) Oy, 02230 Espoo (FI)
(72) Inventor: KROGERUS, Helge, 28100 Pori (FI); MÄKELÄ, Pasi, 28430 Pori (FI)
(74) Representative: Papula Oy
(86) International application number: PCT/FI2016/050821
(87) International publication number: WO 2017/089651

(56) References cited:
- US-A- 4 307 872
- US-A- 4 529 439
- E. C. VANDERSTAAY ET AL: "A computational thermodynamics model of submerged arc electric furnace ferromanganese smelting", TRANSACTIONS - INSTITUTION OF MINING AND METALLURGY. SECTION C.MINERAL PROCESSING AND EXTRACTIVE METALLURGY, vol. 113, no. 1, 18 April 2004 (2004-04-18), pages 38-44, XP055341205, GB ISSN: 0371-9553, DOI: 10.1179/037195504225004706

## Description

### Field of the invention

The invention relates to a method for preheating and smelting manganese ore sinter as defined in the preamble of independent claim 1.

### Objective of the invention

The object of the invention is to provide a method for energy efficient smelting manganese ore sinter.

### Short description of the invention

The method for preheating and smelting manganese ore sinter is characterized by the definitions of independent claim 1.

Preferred embodiments of the method are defined in the dependent claims 2 to 12.

The invention is based on preheating the feed mixture containing at least manganese ore sinter and reducing agent in order to eliminate the moisture from the feed mixture and to preheat the feed mixture to as high a temperature as possible without burning or loosing carbon in the reduction agent required for reduction purposes in the feed mixture.

In preheating of manganese containing, the carbon consuming reactions, especially the Boudouard reaction (C(s) + CO₂(g) ↔ 2CO (g)), is an limiting factor. Water gas reaction occurs also, H₂O + C → H₂ + CO. Thus the preheating temperature in the pre-treatment silo can locally be maximum 600 to 700 °C, depending on the reactivity of the carbon in the reducing agent of the feed mixture. The average temperature of the hot charge to the electric furnace is typically below 600°C.

Preheating of the feed mixture saves electrical energy of the submerged electric arc furnace, improves the operation, improves production and safety of the smelting by preventing reaction between carbon and oxygen in the feed mixture and prevents thus uncontrolled increase of temperature and possible explosions.

### List of figures

In the following the method and the apparatus for preheating and smelting manganese ore sinter will described in more detail by referring to the figures, of which
Figure 1 shows a flow sheet of first embodiment, and
Figure 2 shows a flow sheet of second embodiment.

### Detailed description of the invention

First the method for preheating of smelting manganese ore sinter and some preferred embodiments and variants of the method will be described in greater detail.

The method comprises a feeding step for feeding feed mixture 1 comprising at least manganese ore sinter 2, reducing agent 3 , and fluxing agent 4 into an submerged electric arc furnace 5.

The method comprises a smelting step for smelting said feed mixture 1 in the submerged electric arc furnace 5 to form a layer containing liquid manganese alloy (not shown in the drawings) and a layer containing slag (not shown in the drawings) above the layer containing liquid manganese alloy.

The method comprises a withdrawing step for withdrawing liquid manganese alloy and slag separately or simultaneously from the submerged electric arc furnace 5.

The method comprises a first discharging step for discharging carbon monoxide containing carbonaceous gas 6 from the submerged electric arc furnace 5.

The method comprises a combusting step for combusting carbon monoxide containing carbonaceous gas 6 discharged in the first discharging step from the submerged electric arc furnace 5 in presence of oxygen such as air in a burner 7 to form carbon dioxide containing carbonaceous gas 9.

The feeding step of the method comprises a heating step for heating said feed mixture 1 with said carbon dioxide containing carbonaceous gas 9 formed in the combusting step in a pre-treatment silo 8 prior feeding feed mixture 1 into the submerged electric arc furnace 5.

The submerged electric arc furnace 5 that is used in the method is preferably an alternating current (AC) submerged electric arc furnace 5.

The burner 7 is preferably connected to the pre-treatment silo 8 and the pre-treatment silo 8 is preferably connected to the submerged electric arc furnace 5 so that gases such as oxygen from the ambient air is prevented from entering the burner 7, the pre-treatment silo 9 and the submerged electric arc furnace 5 so as to prevent uncontrolled reactions of said feed material 1.

The manganese ore sinter 9 may have a particle size between 6 and 75 mm.

The method may include heating the feed mixture 1 in the heating step to a temperature in the range between 400 and 700°C preferably to a temperature between 500 and 650°C.

The method includes preferably, but not necessarily, adjusting the temperature of said carbon dioxide containing carbonaceous gas 9 that is used in the heating step. The temperature of the said carbon dioxide containing carbonaceous gas 9 that is used in the heating step may be controlled to a temperature in the range between 600 and 900°C.

In the burner 7, the carbon monoxide containing carbonaceous gas 6 received from the submerged electric arc furnace 5 is preferably burned by an air ratio below 1, such as between 0.9 and 0.95. Oxygen (O₂) content in the carbon dioxide containing carbonaceous gas 9 formed in the combusting step should be very low to minimize the oxidation of carbon in the feed mixture 1. The content of carbon monoxide (CO) and hydrogen (H₂) in the carbon dioxide containing carbonaceous gas 9 formed in the combusting step should be very low for avoiding the explosions in the gas lines especially between the burner 7 and the pre-treatment silo 8 or in the pre-treatment silo 8.

The method may include burning carbon monoxide containing carbonaceous gas 6 discharged from the submerged electric arc furnace 5 by means of butane in the burning step

The method may include burning carbon monoxide containing carbonaceous gas 6 discharged from the submerged electric arc furnace 5 by means of CO gas or e.g. butane (C₄H₁₀) in the burning step so that the molar ratio of air to butane is in the range between 0.9 - 0.95.

The carbon dioxide containing carbonaceous gas 9 that is formed in the combusting step and that is used in the heating step, may containing in percentages of volume:
CO₂: between 25 and 35 %,
N₂: between 50 and 65 %,
H₂O: between 3 and 8 % H₂O
O₂: less than 1 %
H₂: less than 1 %, and
CO: less than 2 %.

The heating step comprises preferably heating said feed mixture 1 by feeding said carbon dioxide containing carbonaceous gas 9 formed in the combusting step into the pre-treatment silo 8. In such case, the heating step includes preferably feeding said carbon dioxide containing carbonaceous gas 9 formed in the combusting step into the pre-treatment silo 8 from below so that carbon dioxide containing carbonaceous gas 9 flows in the opposite direction, such as upwards, with respect the feed mixture in the pre-treatment silo 8.

The method may, as shown in figure 2, include a first scrubbing step of the carbon monoxide gas 6 discharged from the submerged electric arc furnace 5. This is prior burning the carbon monoxide gas 6 in the burner 7.

The method may, as shown in figure 2, include a second discharging step for discharging carbon dioxide containing carbonaceous gas 9 from the pre-treatment silo 8 and for feeding carbon dioxide containing carbonaceous gas 9 discharged from the pre-treatment silo 8 to the burner 7 and/or into the carbon dioxide containing carbonaceous gas 9 that is formed in the combusting step by means of the burner 7 to adjust the temperature of the carbon dioxide containing carbonaceous gas 9 that is formed in the combusting step. In such case, the method may include a second scrubbing step for scrubbing carbon dioxide containing carbonaceous gas 9 discharged in the second discharging step from the pre-treatment silo 8 in a second scrubber 11.

The reducing agent 3 of the feed mixture 1 may contain carbonaceous material such as metallurgical coke, anthracite or charcoal.

The fluxing agent 4 of the feed mixture 1 may contain e.g. calcite, coarse burned lime, quartz, dolomite.

The chemical analysis of the manganese ore sinter 2 is depending on the chemical analysis of manganese ore. Manganese ores are calcium based, carbonate based and oxidized based which of chemical analyses greatly varies. A possible content of the manganese ore sinter 2 is:
Mn: 40 to 55 %,
Fe: 1 to 10 %,
SiO₂: 4 to 10 %
MgO: 0.4 to 8 %
CaO: 1.0 - 15 %
A₂O₃: 1-15 %
K₂O: less than 1.5 %
BaO: less than 0.6 %

Next the apparatus for preheating and smelting manganese ore sinter and some preferred embodiments and variants of the method will be described in greater detail.

The apparatus comprises a submerged electric arc furnace 5 for smelting feed mixture 1 comprising at least manganese ore sinter 2, reducing agent 3, and fluxing agent 4. A layer containing liquid manganese alloy and a layer containing slag above the layer containing liquid manganese alloy are formed in the smelting in the submerged electric arc furnace 5.

The apparatus comprises first feeding means 12 configured to feed said feed mixture 1 into the submerged electric arc furnace 5.

The apparatus comprises withdrawing means 13 for withdrawing liquid manganese and slag separately or simultaneously from the submerged electric arc furnace 5.

The apparatus comprises first discharging means 14 for discharging carbon monoxide containing carbonaceous gas 6 from the submerged electric arc furnace 5.

The apparatus comprises a burner 7 for combusting carbon monoxide containing carbonaceous gas 6 received from the first discharging means 14 in presence of oxygen such as air to form carbon dioxide containing carbonaceous gas 9.

The first feeding means 12 of the apparatus comprises a pre-treatment silo 8 for heating said feed mixture 1 with said carbon dioxide containing carbonaceous gas 9 formed by means of the burner 7 prior feeding said feed mixture 1 into the submerged electric arc furnace 5.

The submerged electric arc furnace 5 in the apparatus is preferably an alternating current (AC) submerged electric arc furnace 5.

The burner 7 is preferably connected to the pre-treatment silo 8 and the pre-treatment silo 8 is preferably connected to the submerged electric arc furnace 5 so that gases such as oxygen from the ambient air is prevented from entering the burner 7, the pre-treatment silo 9 and the submerged electric arc furnace 5 so as to prevent uncontrolled reactions of said feed material 1.

The manganese ore sinter 9 may have a particle size between 6 and 75 mm.

The pre-treatment silo 8 of the apparatus may be configured to heat the feed mixture 1 to a temperature in the range between 400 and 700°C, preferable to a temperature in the range between 500 and 650°C.

The apparatus comprises preferably, but not necessarily, gas temperature adjusting means (not shown in the figures) configured to adjust the temperature of said carbon dioxide containing carbonaceous gas 9 prior feeding said carbon dioxide containing carbonaceous gas 9 to the pre-treatment silo 8. The temperature of the feed carbon dioxide containing carbonaceous gas 9 that is fed to the pre-treatment silo 8 may be controlled to the range between 600 and 900°C.

In the burner 7, the carbon monoxide containing carbonaceous gas 6 received from the submerged electric arc furnace 5 is preferably burned by an air ratio below 1, such as between 0.9 and 0.95. Oxygen (O₂) content in the carbon dioxide containing carbonaceous gas 9 formed in the combusting step should be very low to minimize the oxidation of carbon in the feed mixture 1. The content of carbon monoxide (CO) and hydrogen (H₂) in the carbon dioxide containing carbonaceous gas 9 formed in the combusting step should be very low for avoiding the explosions in the gas lines or in the pre-treatment silo 8.

The burner 7 may be a CO, a butane, and a LPG burner.

Said carbon dioxide containing carbonaceous gas 9, that is produced by the burner 7 contains preferably, but not necessarily, in percentages of volume
CO₂: between 25 and 35 %,
N2: between 50 and 65 %,
H₂O: between 5 and 15 % H₂O
O2: less than 1 %
H₂: less than 1 %, and
CO: less than 2 %

The arrangement, preferably the burner 7, is preferably configured to feed said carbon dioxide containing carbonaceous gas 9 into the pre-treatment silo 8 from below so that said carbon dioxide containing carbonaceous gas 9 flows upwards in the pre-treatment silo 8 through the feed mixture.

The apparatus may, as shown in figure 2, comprise a first scrubber 10 configured to scrub carbon monoxide containing carbonaceous gas 6 discharged from the electric arc furnace 5 prior combusting carbon monoxide to the burner 7.

The apparatus may, as shown in figure 2, comprise second discharging means 15 configured to discharge carbon dioxide containing carbonaceous gas 9 from the pre-treatment silo 8 and third feeding means (not marked with a reference numeral) configured to feed carbon dioxide containing carbonaceous gas 9 discharged from the second discharging means 15 to the burner 7 and/or to into carbon dioxide containing carbonaceous gas 9 formed by the burner 7 to adjust the temperature of the carbon dioxide containing carbonaceous gas 9 formed by the burner 7.

The second discharging means 15 of the apparatus may, as shown in figure 2, comprise a second scrubber 11 configured to scrub carbon dioxide containing carbonaceous gas 9 discharged from the pre-treatment silo 8. Cold and scrubbed gases removed from the carbon dioxide containing carbonaceous gas 9 in the second scrubber 11 may be used in the optional temperature adjustment means for adjusting the temperature of the carbon dioxide containing carbonaceous gas 9 that is fed to the pre-treatment silo 8.

The first feeding means 12 of the apparatus may be configured to feed reducing agent 3 containing carbonaceous material such as metallurgical coke, anthracite and/or charcoal.

The first feeding means 12 of the apparatus may be configured to feed fluxing agent 4 containing at least one of calcite, coarse burned lime, dolomite and quartz.

The first feeding means 12 of the apparatus may be configured to feed manganese ore sinter 2 containing in percentages of mass:
Mn: 40 to 55 %.
Fe: 1 to 10 %,
SiO₂: 4 to 10 %
MgO: 0.4 to 8 %
CaO: 1 to 15 %
A₂O₃: 1 to 15 %
K₂O: less than 1.5 %, and
BaO: less than 0.6 %

The first feeding means 12 may, as shown in figure 2, comprise a silo arrangement 16 comprising a first silo 17 for manganese ore sinter 2, a second silo 18 for reducing agent 3, and a third silo 19 for fluxing agent 4.

### Example 1

Metallurgical coke having the composition defined in table 1 and calcite manganese ore sinter having the composition defined in column "Original sinter" in table 2 was mixed in ratio 80 percentages by weight (wt.%) calcite ore and 20 wt.% and heated in a vessel to four different temperatures: 500°C, 600°C, 700°C and 800°C. The calcite manganese ore sinter was prior the mixing crushed and sieved into a particle size of 2.38 to 6.73 mm and the metallurgical coke was prior the mixing crushed and sieved into a particle size of 0.595 to 4.76 mm

The heating was performed by induction heating and gas containing carbon dioxide and nitrogen in ratio 30% carbon dioxide and 70% was blown into the vessel to simulate actual heating conditions.

The composition of the calcite manganese ore sinter was measured in each case: 500°C, 600°C, 700°C and 800°C. As can be seen from columns "500°C"," 600°C", "700°C" and "800°C" table 3, the change in the composition of the calcite manganese ore sinter was only marginal, which means for example that hardly any reduction of the oxides occurred.

**Table 1. Chemical analysis of metallurgical coke**

| | | Coke wt. % | Ash, wt. % |
|---|---|---|---|
| C | Leco ¹⁾ | 84 | |
| C_{fix} ⁶⁾ | kem. ²⁾ | 85 | |
| S | Leco ¹⁾ | 0.78 | |
| Volatiles | kem. | 1.2 | |
| ash | kem. | 12.7 | |
| Fe | ICP ³⁾ | 0.61 ⁴⁾ | 4.8 |
| SiO₂ | kem. | 7.14 ⁴⁾ | 56.2 |
| CaO | ICP ³⁾ | 0.23 ⁴⁾ | 1.8 |
| MgO | ICP ³⁾ | 0.24 ⁴⁾ | 1.9 |
| Al₂O₃ | ICP ³⁾ | 3.07 ⁴⁾ | 24.2 |

| | | | |
|---|---|---|---|
| ¹⁾ Leco on C, S -analyzer ²⁾ by wet chemically ³⁾ ICP (plasma emission spectrometer) ⁴⁾ wt. % of the coke ⁵⁾ ash amount in coke is 12.7 wt. % ⁶⁾ C_{fix} - value: 100 % - (volatiles + ash + sulphur) | | | |

**Table 2. Chemical analysis of the preheated sinters of calcite ore as function of preheating temperature**

| Component | Original sinter | 500°C | 600°C | 700°C | 800°C |
|---|---|---|---|---|---|
| Mn | 43.7 | 43.9 | 44.5 | 44.5 | 4.42 |
| C | 0.07 | 0.05 | 0.05 | 0.04 | 0.04 |
| Fe | 5.2 | 5.2 | 5.1 | 5,2 | 5.0 |
| SiO₂ | 8.2 | 8.0 | 7.5 | 7.6 | 7.8 |
| MgO | 4.5 | 4.7 | 4.8 | 4.7 | 4.5 |
| CaO | 15.2 | 15.2 | 14.7 | 14.6 | 15.0 |
| Al₂O₃ | 0.71 | 0.72 | 0.68 | 0.71 | 0.68 |
| K₂O | 0.02 | 0.01 | 0.02 | 0.02 | 0.01 |
| BaO | 0.24 | 0.24 | 0.24 | 0.23 | 0.24 |
| TiO₂ | 0.04 | 0.04 | 0.04 | 0.03 | 0.03 |
| P₂O₅ | < 0.03 | < 0.03 | < 0.03 | < 0.03 | < 0.03 |
| CoO | 0.01 | 0.01 | 0.01 | 0.01 | 0.01 |
| Cr₂O₃ | 0.03 | 0.03 | 0.03 | 0.03 | 0.03 |
| CuO | < 0.01 | < 0.01 | < 0.01 | < 0.01 | < 0.01 |
| NiO | < 0.01 | < 0.01 | < 0.01 | < 0.01 | < 0.01 |
| ZnO | 0.01 | 0.01 | 0.01 | 0.01 | 0.01 |
| Fe ¹⁾ | 0.44 | 0.39 | 0.36 | 0.39 | 0.37 |

| | | | | | |
|---|---|---|---|---|---|
| ¹⁾ Metallic amount | | | | | |

### Example 2

Metallurgical coke having the composition defined in table 1 and oxidized manganese ore sinter having the composition defined in column "Original sinter" in table 3 was mixed in ratio 80 wt.% calcite ore and 20 wt.% charcoal and heated in a vessel to four different temperatures: 500°C, 600°C, 700°C and 800°C. The oxidized manganese ore sinter was prior the mixing crushed and sieved into a particle size of 2.38 to 6.73 mm and the metallurgical coke was prior the mixing crushed and sieved into a particle size of 0.595 to 4.76 mm.

The heating was performed by induction heating and gas containing carbon dioxide and nitrogen in ratio 30% carbon dioxide and 70% was blown into the vessel to simulate actual heating conditions.

The composition of the oxidized manganese ore sinter was measured in each case: 500°C, 600°C, 700°C and 800°C. As can be seen from columns "500°C"," 600°C", "700°C" and "800°C" table 3, the change in the composition of the oxidized manganese ore sinter was only marginal, which means for example that hardly any reduction of the oxides occurred.

**Table 3. Chemical analysis of the preheated sinters of oxidized ore as function of preheating temperature**

| Component | Original sinter | 500°C | 600°C | 700°C | 800°C |
|---|---|---|---|---|---|
| Mn | 59.0 | 60.8 | 58.9 | 59.8 | 59.7 |
| C | 0.03 | 0.03 | 0.03 | 0.15 | 0.04 |
| Fe | 2.7 | 2.6 | 3.1 | 2.7 | 3.0 |
| SiO₂ | 3.4 | 3.4 | 3.3 | 3.4 | 3.1 |
| MgO | 0.28 | 0.24 | 0.41 | 0.26 | 0.39 |
| CaO | 0.62 | 0.66 | 0.53 | 0.58 | 0.66 |
| Al₂O₃ | 6.0 | 5.9 | 5.8 | 5.9 | 5.7 |
| K₂O | 0.87 | 0.97 | 0.83 | 0.90 | 0.84 |
| BaO | 0.28 | 0.28 | 0.29 | 0.27 | 0.30 |
| TiO₂ | 0.17 | 0.17 | 0.16 | 0.17 | 0.16 |
| P₂O₅ | 0.18 | 0.21 | 0.20 | 0.20 | 0.16 |
| CoO | 0.17 | 0.18 | 0.18 | 0.18 | 0.17 |
| Cr₂O₃ | 0.32 | 0.22 | 1.0 | 0.28 | 0.86 |
| CuO | 0.06 | 0.06 | 0.06 | 0.06 | 0.06 |
| NiO | 0.04 | 0.04 | 0.04 | 0.04 | 0.04 |
| ZnO | 0.06 | 0.06 | 0.06 | 0.06 | 0.06 |
| Fe ¹⁾ | 0.57 | 0.53 | 0.37 | 0.35 | 0.42 |

| | | | | | |
|---|---|---|---|---|---|
| ¹⁾ metallic amount | | | | | |

### Example 3

In an apparatus according to figure 2, manganese sinter as defined in table 4 was fed at a feed rate of 131 kg/h, and reducing agent as defined in row "charcoal" in table 5 was fed at a feed rate of 24 kg/h into the pre-treatment silo 8. Carbonaceous gas containing 57 vol-% N₂, 30 vol.%, CO₂ and 11 vol.% H₂O and having a temperature of 850°C was fed at a feed rate of 970 m³/h into the pre-treatment silo 8.

**Table 4: Chemical analysis of the manganese sinter, wt.%**

| Component | Analysis, wt. % |
|---|---|
| Mn | 50.2 |
| Fe ₜₒₜₐₗ | 6.6 |
| Fe ²⁺ | < 0.05 |
| Fe _{metallic} | < 0.1 |
| SiO₂ | 6.7 |
| CaO | 1.0 |
| MgO | 0.43 |
| A₂O₃ | 13.2 |
| K | 1.2 |
| Ba | 0.43 |
| C-ₜₒₜₐₗ (volatiles) | 0.03 |
| H₂O | 0.26 |

**Table 5. Chemical analysis of reducing agents in examples 3 and 4, wt. %.**

| Component | Charcoal | Coke |
|---|---|---|
| C ₜₒₜₐₗ | 75 | |
| C_{fix} | 72 | 85.0 |
| Volatiles | 26 | 3.0 |
| ASH | 2.3 | 10.2 |
| S | 0.01 | 0.65 |

| Analysis of volatiles of charcoal | | |
|---|---|---|
| H₂ | 24.6 | |
| O₂ | 0.1 | |
| N₂ | 0.5 | |
| CO | 36.9 | |
| CO₂ | 16.5 | |
| CH₄ | 21.4 | |
| H₂O | 8.0 | |

Carbon components of charcoal starts to gasify at 450°C.

It was observed that a mixture of where charcoal is used as reducing agent 3 can be preheated to a temperature of 400°C without the carbon gasification. The charcoal starts to oxidize either through the Boudouard reaction or through the water-gas-reaction. In addition, the oxygen content and the water in the carbon dioxide containing carbonaceous gas 9 should be low to avoid oxidizing of the carbon.

### Example 4

In an apparatus according to figure 2, manganese sinter as defined table 4 was fed at a feed rate of 131 kg/h, and reducing agent as defined in row "Coke" in table 5 was fed at a feed rate of 24 kg/h into the pre-treatment silo 8. Carbonaceous gas containing 57 vol-% N₂, 30 vol-%, CO₂ and 11 vol.% H₂O and having a temperature of 850°C was fed at a feed rate of 970 m³/h into the pre-treatment silo 8

Carbon of coke starts to gasify at 700°C.

It was observed that a mixture of where coke is used as reducing agent 3 can be preheated to a temperature of 650°C without the carbon in the coke starts to oxidize either through the Boudouard reaction or through the water-gas-reaction. In addition, the oxygen content and the water in the carbon dioxide containing carbonaceous gas 9 should be low to avoid oxidizing of the carbon.

It is apparent to a person skilled in the art that as technology advanced, the basic idea of the invention can be implemented in various ways. The invention and its embodiments are therefore not restricted to the above examples, but they may vary within the scope of the claims.

## Claims

1. A method for preheating and smelting manganese ore sinter, **characterized**
**by** a feeding step for feeding feed mixture (1) containing at least manganese ore sinter (2), reducing agent (3), and fluxing agent (4) into an submerged electric arc furnace (5),
by a smelting step for smelting feed mixture (1) in the submerged electric arc furnace (5) to form a layer containing liquid manganese alloy and a layer containing slag above the layer containing liquid manganese alloy,
by a withdrawing step for withdrawing liquid manganese and slag from the submerged electric arc furnace (5),
by a first discharging step for discharging carbon monoxide containing carbonaceous gas (6) from the submerged electric arc furnace (5),
by a combusting step for combusting carbon monoxide containing carbonaceous gas (6) discharged from the submerged electric arc furnace (5) in the first discharging step in presence of oxygen such as air in a burner (7) to form carbon dioxide containing carbonaceous gas (9),
by a heating step for heating said feed mixture (1) in a pre-treatment silo (8) to a temperature in the range between 400 and 700°C prior feeding said feed mixture (1) into the submerged electric arc furnace (5) with said carbon dioxide containing carbonaceous gas (9) formed in the combusting step,
by a second discharging step for discharging carbon dioxide containing carbonaceous gas (9) from the pre-treatment silo (8),
by feeding carbon dioxide containing carbonaceous gas (9) discharged in the second discharging step to the burner (7) and/or into carbon dioxide containing carbonaceous gas (9) that is used in the heating step to adjust the temperature of the carbon dioxide containing carbonaceous gas (9) formed in the combusting step, and
by heating the feed mixture (1) in the heating step by feeding said carbon dioxide containing carbonaceous gas (9) into the pre-treatment silo (8).

2. The method according to claim 1, **characterized**
**by** the submerged electric arc furnace (5) being an alternating current (AC) submerged electric arc furnace (5) .

3. The method according to claim 1 or 2, **characterized**
**by** the manganese ore sinter (2) having a particle size between 6 and 75 mm.

4. The method according to any of the claims 1 to 3, **characterized**
**by** heating the feed mixture (1) in the pre-treatment silo (8) in the heating step to a temperature in the range between 500 and 650°C.

5. The method according to any of the claims 1 to 4, **characterized**
**by** adjusting the temperature of said carbon dioxide containing carbonaceous gas (9) that is used in the heating step to a temperature in the range between 580 and 900°C.

6. The method according to any of the claims 1 to 5, **characterized** said carbon dioxide containing carbonaceous gas (9) that is used in the heating step containing in percentages of volume:
CO₂: between 25 and 35 %,
N₂: between 50 and 65 %,
H₂O: between 3 and 8 %
O₂: less than 1 %
H₂: less than 1 %, and
CO: less than 2 %.

7. The method according to any of claims 1 to 6, **characterized**
**by** feeding said carbon dioxide containing carbonaceous gas (9) into the pre-treatment silo (8) in the heating step from below so that said carbon dioxide containing carbonaceous gas (9) flows upwards in the pre-treatment silo (8) through the feed mixture (1) in the pre-treatment silo (8).

8. The method according to any of the claims 1 to 7, **characterized**
**by** scrubbing carbon monoxide containing carbonaceous gas (6) discharged in the first discharging step from the submerged electric arc furnace (5) in a first scrubber (10) prior feeding carbon monoxide containing carbonaceous gas (6) discharged in the first discharging step to the burner (7).

9. The method according to any of the claims 1 to 8, **characterized**
**by** scrubbing carbon dioxide containing carbonaceous gas (9) discharged in the second discharging step in a second scrubber (11) prior feeding carbon dioxide containing carbonaceous gas (9) discharged in the second discharging step to the burner (7).

10. The method according to any of the claims 1 to 9, **characterized**
**by** the reducing agent (3) containing carbonaceous material such as coke, anthracite, and/or charcoal.

11. The method according to any of the claims 1 to 10, **characterized**
**by** the fluxing agent (4) containing at least one of calcite, coarse burned lime, dolomite and quartz.

12. The method according to any of the claims 1 to 11, **characterized**
**by** the manganese ore sinter (2) containing in percentages of mass:
Mn: 40 to 55 %,
Fe: 1 to 10 %,
SiO₂: 4 to 10 %
MgO: 0.4 to 8 %
CaO: 1 to 15 %
A₂O₃: 1 to 15 %
K₂O: less than 1.5 %, and
BaO: less than 0.6 %

## Patentansprüche

1. Verfahren zum Vorwärmen und Schmelzen von Manganerzsinter, **gekennzeichnet**
**durch** eine Zufuhrstufe zum Zuführen eines Zufuhrgemisches (1), das mindestens Manganerzsinter (2), Reduktionsmittel (3) und Flussmittel (4) enthält in einen Elektroreduktionsofen (5),
durch eine Schmelzstufe zum Schmelzen des Zufuhrgemisches (1) im Elektroreduktionsofen (5) unter Bildung einer Schicht enthaltend flüssige Manganlegierung und einer Schicht enthaltend Schlacke, die über der Schicht enthaltend flüssige Manganlegierung liegt,
durch eine Entnahmestufe zur Entnahme von flüssigem Mangan und Schlacke aus dem Elektroreduktionsofen (5),
durch eine erste Austragungsstufe zum Austragen von Kohlenmonoxid enthaltendem, kohlenstoffhaltigem Gas (6) aus dem Elektroreduktionsofen (5),
durch eine Verbrennungsstufe zum Verbrennen von aus dem Elektroreduktionsofen (5) bei der ersten Austragungsstufe ausgetragenen, Kohlenmonoxid enthaltenden, kohlenstoffhaltigen Gases (6) in Gegenwart von Sauerstoff, wie Luft, in einem Brenner (7) unter Bildung von Kohlendioxid enthaltendem, kohlenstoffhaltigem Gas (9),
durch eine Erwärmungsstufe zum Erwärmen des Zufuhrgemisches (1) in einem Vorbehandlungssilo (8) auf eine Temperatur im Bereich von 400 bis 700 °C vor dem Zuführen des Zufuhrgemisches (1) in den Elektroreduktionsofen (5) mit dem in der Verbrennungsstufe gebildeten, Kohlendioxid enthaltenden, kohlenstoffhaltigen Gas (9),
durch eine zweite Austragungsstufe zum Austragen von Kohlendioxid enthaltendem, kohlenstoffhaltigem Gas (9) aus dem Vorbehandlungssilo (8),
durch Zuführen von in der zweiten Austragungsstufe ausgetragenen, Kohlendioxid enthaltendem, kohlenstoffhaltigem Gas (9) in den Brenner (7) und/oder in das Kohlendioxid enthaltende, kohlenstoffhaltige Gas (9), das in der Erwärmungsstufe zur Einstellung der Temperatur des in der Verbrennungsstufe gebildeten, Kohlendioxid enthaltenden, kohlenstoffhaltigen Gases (9) verwendet wird, und
durch Erwärmen des Zufuhrgemisches (1) in der Erwärmungsstufe durch Zuführen des Kohlendioxid enthaltenden, kohlenstoffhaltigen Gases (9) in den Vorbehandlungssilo (8).

2. Verfahren nach Anspruch 1, **dadurch gekennzeichnet,**
**dass** es sich beim Elektroreduktionsofen (5) um einen Wechselstrom (AC)-Elektroreduktionsofen (5) handelt.

3. Verfahren nach Anspruch 1 oder 2, **dadurch gekennzeichnet,**
**dass** der Manganerzsinter (2) eine Teilchengröße von 6 bis 75 mm aufweist.

4. Verfahren nach einem der Ansprüche 1 bis 3, **gekennzeichnet,**
**durch** Erwärmen des Zufuhrgemisches (1) bei der Erwärmungsstufe im Vorbehandlungsilo (8) auf eine Temperatur im Bereich von 500 bis 650 °C.

5. Verfahren nach einem der Ansprüche 1 bis 4, **gekennzeichnet,**
**durch** Einstellen der Temperatur des in der Erwärmungsstufe verwendeten, Kohlendioxid enthaltenden, kohlenstoffhaltigen Gases (9) auf eine Temperatur im Bereich von 580 bis 900 °C.

6. Verfahren nach einem der Ansprüche 1 bis 5, **dadurch gekennzeichnet, dass** das in der Erwärmungsstufe verwendete, Kohlendioxid enthaltende, kohlenstoffhaltige Gas (9) folgende Bestandteile (in Vol-%) enthält
| | |
|---|---|
| CO₂: | 25 bis 35 %, |
| N₂: | 50 bis 65 %, |
| H₂O | 3 bis 8 %, |
| O₂: | weniger als 1 %, |
| H₂: | weniger als 1 % und |
| CO: | weniger als 2 %. |

7. Verfahren nach einem der Ansprüche 1 bis 6, **gekennzeichnet,**
**durch** Zuführen des Kohlendioxid enthaltenden, kohlenstoffhaltigen Gases (9) bei der Erwärmungsstufe in den Vorbehandlungsilo (8) von unten, so dass das Kohlendioxid enthaltende, kohlenstoffhaltige Gas (9) in Richtung nach oben in das Vorbehandlungsilo (8) durch das Zufuhrgemisch (1) im Vorbehandlungsilo (8) strömt.

8. Verfahren nach einem der Ansprüche 1 bis 7, **gekennzeichnet,**
**durch** Waschen des in der ersten Austragungsstufe aus dem Elektroreduktionsofen (5) ausgetragenen, Kohlenmonoxid enthaltenden, kohlenstoffhaltigen Gases (6) in einem ersten Gaswäscher (10), bevor das in der ersten Austragungsstufe ausgetragene, Kohlenmonoxid enthaltende, kohlenstoffhaltige Gas (6) dem Brenner (7) zugeführt wird.

9. Verfahren nach einem der Ansprüche 1 bis 8, **gekennzeichnet,**
**durch** Waschen des in der zweiten Austragungsstufe ausgetragenen, Kohlendioxid enthaltenden, kohlenstoffhaltigen Gases (9) in einem zweiten Gaswäscher (11), bevor das in der zweiten Austragungsstufe ausgetragene, Kohlendioxid enthaltende, kohlenstoffhaltige Gas (9) dem Brenner (7) zugeführt wird.

10. Verfahren nach einem der Ansprüche 1 bis 9, **dadurch gekennzeichnet, dass** das Reduktionsmittel (3) ein kohlenstoffhaltiges Material, wie Koks, Anthrazit und/oder Holzkohle, enthält.

11. Verfahren nach einem der Ansprüche 1 bis10, **dadurch gekennzeichnet, dass** das Flussmittel (4) mindestens einen der Bestandteile Calcit, groben gebrannten Kalk, Dolomit und Quarz enthält.

12. Verfahren nach einem der Ansprüche 1 bis 11, **dadurch gekennzeichnet, dass** der Manganoxidsinter (2) in Massenprozent enthält
| | |
|---|---|
| Mn: | 40 bis 55 %, |
| Fe: 1 | bis 10%, |
| SiO₂: | 4 bis 10%, |
| MgO: | 0,4 bis 8 %, |
| CaO: | 1 bis 15%, |
| A₂O₃: | 1 bis 15 %, |
| K₂O: | weniger als 1,5 % und |
| BaO: | weniger als 0,6 %. |

## Revendications

1. Procédé pour préchauffer et fondre une fritte de minerai de manganèse, **caractérisé**
**par** une étape d'alimentation pour introduire un mélange d'alimentation (1) contenant au moins une fritte de minerai de manganèse (2), un agent réducteur (3) et un fondant (4) dans un four à arc électrique immergé (5),
par une étape de fusion pour fondre le mélange d'alimentation (1) dans le four à arc électrique immergé (5) pour former une couche contenant un alliage de manganèse liquide et une couche contenant des scories au-dessus de la couche contenant un alliage de manganèse liquide,
par une étape de retrait pour retirer le manganèse liquide et les scories hors du four à arc électrique immergé (5),
par une première étape de décharge pour décharger un gaz carboné contenant du monoxyde de carbone (6) hors du four à arc électrique immergé (5),
par une étape de combustion pour brûler le gaz carboné contenant du monoxyde de carbone (6) déchargé hors du four à arc électrique immergé (5) dans la première étape de décharge en présence d'oxygène tel que de l'air dans un brûleur (7) pour former un gaz carboné contenant du dioxyde de carbone (9),
par une étape de chauffage pour chauffer ledit mélange d'alimentation (1) dans un silo de prétraitement (8) à une température située dans la plage comprise entre 400 et 700°C avant l'introduction dudit mélange d'alimentation (1) dans le four à arc électrique immergé (5) avec ledit gaz carboné contenant du dioxyde de carbone (9) formé dans l'étape de combustion,
par une deuxième étape de décharge pour décharger le gaz carboné contenant du dioxyde de carbone (9) hors du silo de prétraitement (8),
par l'introduction du gaz carboné contenant du dioxyde de carbone (9) déchargé dans la deuxième étape de décharge dans le brûleur (7) et/ou dans le gaz carboné contenant du dioxyde de carbone (9) utilisé dans l'étape de chauffage pour ajuster la température du gaz carboné contenant du dioxyde de carbone (9) formé dans l'étape de combustion, et
par le chauffage du mélange d'alimentation (1) dans l'étape de chauffage par introduction dudit gaz carboné contenant du dioxyde de carbone (9) dans le silo de prétraitement (8).

2. Procédé selon la revendication 1, **caractérisé en ce que** le four à arc électrique immergé (5) est un four à arc électrique immergé (5) en courant alternatif (AC) .

3. Procédé selon la revendication 1 ou 2, **caractérisé en ce que** la fritte de minerai de manganèse (2) a une granulométrie comprise entre 6 et 75 mm.

4. Procédé selon l'une quelconque des revendications 1 à 3, **caractérisé par** le chauffage du mélange d'alimentation (1) dans le silo de prétraitement (8) dans l'étape de chauffage à une température située dans la plage comprise entre 500 et 650°C.

5. Procédé selon l'une quelconque des revendications 1 à 4, **caractérisé par** l'ajustement de la température dudit gaz carboné contenant du dioxyde de carbone (9) qui est utilisé dans l'étape de chauffage à une température située dans la plage comprise entre 580 et 900°C.

6. Procédé selon l'une quelconque des revendications 1 à 5, **caractérisé en ce que** ledit gaz carboné contenant du dioxyde de carbone (9) qui est utilisé dans l'étape de chauffage contient, en pourcentages en volume :
CO₂ : entre 25 et 35 %,
N₂ : entre 50 et 65 %,
H₂O : entre 3 et 8 %,
O₂ : moins de 1 %,
H₂ : moins de 1 %, et
CO : moins de 2 %.

7. Procédé selon l'une quelconque des revendications 1 à 6, **caractérisé par** l'introduction dudit gaz carboné contenant du dioxyde de carbone (9) dans le silo de prétraitement (8) dans l'étape de chauffage depuis le dessous de façon que ledit gaz carboné contenant du dioxyde de carbone (9) circule vers le haut dans le silo de prétraitement (8) à travers le mélange d'alimentation (1) dans le silo de prétraitement (8).

8. Procédé selon l'une quelconque des revendications 1 à 7, **caractérisé par** l'épuration du gaz carboné contenant du monoxyde de carbone (6) déchargé dans la première étape de décharge depuis le four à arc électrique immergé (5) dans un premier épurateur (10) avant l'introduction dans le brûleur (7) du gaz carboné contenant du monoxyde de carbone (6) déchargé dans la première étape de décharge.

9. Procédé selon l'une quelconque des revendications 1 à 8, **caractérisé par** l'épuration du gaz carboné contenant du dioxyde de carbone (9) déchargé dans la deuxième étape de décharge dans un deuxième épurateur (11) avant l'introduction dans le brûleur (7) du gaz carboné contenant du dioxyde de carbone (9) déchargé dans la deuxième étape de décharge.

10. Procédé selon l'une quelconque des revendications 1 à 9, **caractérisé en ce que** l'agent réducteur (3) contient un matériau carboné tel que le coke, l'anthracite et/ou le charbon.

11. Procédé selon l'une quelconque des revendications 1 à 10, **caractérisé en ce que** le fondant (4) contient au moins l'un parmi la calcite, la chaux surcuite grossière, la dolomite et le quartz.

12. Procédé selon l'une quelconque des revendications 1 à 11, **caractérisé en ce que** la fritte de minerai de manganèse (2) contient, en pourcentages en masse :
Mn : 40 à 55 %,
Fe : 1 à 10 %
SiO₂ : 4 à 10 %,
MgO : 0,4 à 8 %,
CaO : 1 à 15 %,
A₂O₃ : 1 à 15 %,
K₂O : moins de 1,5 %, et
BaO : moins de 0,6 %.
